

Aug. 19, 1952

W. A. BATES

2,607,479

AGGLOMERATE TABLING OF TUNGSTEN BEARING ORES

Filed Feb. 4, 1948

2 SHEETS—SHEET 1



INVENTOR  
William A. Bates

BY

*J. M. Adams*  
*G. L. Snow*  
*J. F. Latoff-Roeg*

ATTORNEYS

FIG. 1

Aug. 19, 1952

W. A. BATES

2,607,479

AGGLOMERATE TABLING OF TUNGSTEN BEARING ORES

Filed Feb. 4, 1948

2 SHEETS—SHEET 2



FIG. 2A

SHAKING TABLE

FIG. 2



STRATIFICATION  
BETWEEN RIFFLES

FIG. 3



DISTRIBUTION OF MATERIAL  
BY CONVENTIONAL TABLING

FIG. 4



STRATIFICATION BETWEEN RIFFLES  
IN AGGLOMERATE TABLING

FIG. 5



DISTRIBUTION OF SCHEELITE  
ON SHAKING TABLE

FIG. 6

INVENTOR

William A. Bates

BY J. MacLean

R. L. Snow

P. Filatoff-Noy

ATTORNEYS

Patented Aug. 19, 1952

2,607,479

# UNITED STATES PATENT OFFICE

2,607,479

## AGGLOMERATE TABLING OF TUNGSTEN BEARING ORES

William A. Bates, Berkeley, Calif., assignor to California Research Corporation, San Francisco, Calif., a corporation of Delaware

Application February 4, 1948, Serial No. 6,223

3 Claims. (Cl. 209—49)

1

This invention pertains to a process for beneficiating tungsten-bearing minerals, and more particularly to a froth flotation process for beneficiating scheelite.

It is well known that tungsten-bearing minerals, such as scheelite, are commonly found associated with other minerals of metalliferous and non-metalliferous nature. Thus, a typical scheelite-bearing ore may comprise chalcopyrite and molybdenite, as well as a mixed gangue of calcite, fluorite and the like, and a considerable proportion of siliceous compounds, for example, quartz, garnet and epidote. No difficulty is encountered in separating simultaneously chalcopyrite and molybdenite by froth flotation from such an ore. The combined chalcopyrite-molybdenite concentrate is then readily retreaded to yield separate copper and molybdenum concentrates by any method suitable for the flotation of sulfide minerals. The tailings which are obtained from the flotation of combined chalcopyrite-molybdenite concentrate contain scheelite, calcite, fluorite and siliceous materials.

However, the recovery of scheelite from these tailings is not as satisfactory and straightforward as the above mentioned separation of copper and molybdenum minerals from the chalcopyrite-molybdenite concentrate. As a matter of fact, the application of conventional froth flotation with anionic collectors such as soaps of fatty acids, for example, of tallol acids, for the recovery of scheelite results in an unduly low grade of the tungsten-bearing concentrate (only 10% to 12% by weight of  $WO_3$ ). The unsatisfactory grade of the concentrate is caused by very similar floatabilities of scheelite, calcite and fluorite, all of which have a common calcium ion and a similar chemical constitution. Calcite and fluorite tend to float with scheelite, as do some of the siliceous constituents of the ore pulp, and thus render the production of high grade tungsten-bearing concentrates difficult and costly.

It is the primary object of the present invention to provide a process for the recovery of tungsten-bearing minerals by selective froth flotation from concomitant metalliferous and non-metalliferous contaminants in improved yield and substantially high concentration.

It is a further object of this invention to provide a process for the recovery of tungsten-bearing minerals by selective froth flotation thereof from ores which, in addition to salts of tungsten acids, comprise salts of other acids with the same or an equivalent metal ion.

Another important object of the present invention is to provide a new and efficient process for the selective froth flotation of ores by the application of an improved collector combination which enhances the selectivity of the flotation process.

2

An additional important object of the invention is to provide a new process for beneficiating and recovering tungsten-bearing minerals, which involves carrying out the flotation of said minerals under controlled conditions of pH in order to insure selective flotation thereof from other components of the ore pulp.

Still another particular object of the invention is to provide a new and efficient process for the recovery of high-grade tungsten-bearing minerals from metalliferous and non-metalliferous contaminants thereof by selective froth flotation and by subsequent tabling of the floated tungsten agglomerate.

A more specific object of the present invention is to provide a process for the recovery of high-grade scheelite from an ore pulp containing various metalliferous and non-metalliferous contaminants, such as calcite, fluorite and silicates, by selective froth flotation based on the application of a particular effective collector composition comprising a naphthenic acid, or its soap, and a neutral oil, while controlling the pH of the ore pulp.

Other objects of the invention will become obvious to those skilled in the art from the description which follows.

When a conventional soap collector, such as a tallol soap, is used to beneficiate scheelite in froth flotation, this latter floats readily when the pH of the ore pulp containing it is equal to about 10.0. However, the optimum pH range for the flotation of calcite and fluorite also lies in the neighborhood of this figure, and as a result scheelite does not separate from the other constituents of the pulp. On the other hand, it is observed that in the pH range of about 11.5, and even at a pH of about 11.2, all three minerals: scheelite, calcite and fluorite, are simultaneously depressed in the presence of a soap collector, and flotation of neither can be achieved.

It has now been discovered that scheelite can be effectively separated from calcite, fluorite and most of the siliceous gangue in froth flotation by adjusting the pH of the pulp to a value higher than about 10.5, and preferably between about 10.8 and about 11.5 and even higher, and applying a collector combination comprising a naphthenic acid, conveniently added in the form of a soap, for example, as a sodium soap, and a neutral hydrocarbon oil to effect the selective flotation of scheelite.

This regulation of pH coupled with the addition of neutral hydrocarbon oil to the naphthenic acid collector results in considerable improvement of the grade of final scheelite concentrate by as much as 30% and even higher by weight of  $WO_3$  as compared with scheelite concentrates heretofore obtained in the industry.

Pure naphthenic acids having acid numbers from about 160 to about 190 maximum on oil-free basis may be used in the preparation of collector combinations of the present invention.

Ordinarily, however, the naphthenic acids used as collectors in froth flotation of tungsten-bearing minerals are not pure but contain from about 20% to about 50% by weight of unsaponifiable hydrocarbons or neutral oil based on the combined weight of oil-free acid and oil.

Neutral hydrocarbon oils may be added to these oil-containing naphthenic acids, as well as to pure acids, to secure the improved flotation effects of the present invention, provided the total content of neutral hydrocarbon oil in the collector combination does not exceed 50% by weight of the combined weight of oil-free acid and oil. These oils are preferably petroleum distillates, such as light fuel oils, boiling between about 350° F. and about 700° F. and having a flash point in the range from about 100° F. to about 250° F. and a viscosity less than about 55 S. S. U. at 100° F.

In applying naphthenic acids or their soaps for preparing the collector of the present invention to secure the best flotation results, effective proportions of neutral oil for enhancing the selective flotation of ore may be varied from about 20% to about 50% by weight of the oil, based on the total weight of the oil-free acid and oil in the combination.

The true mechanism responsible for the depression of calcite, fluorite and siliceous gangue and for the selective flotation of scheelite is not fully understood, but it is believed that in the presence of the effective naphthenic acid soap collector, a mono-ionic coating of collector adheres to the surface of mineral particles, and, in turn, adsorbs a second coating or layer of collector ions oriented reversely to the original layer, that is, with polar groups outwardly. This causes the mineral particles to become hydrophilic and unfloatable. However, in the particular pH range of the present invention from 10.8 to 11.5 and higher, the formation of this second layer of soap collector molecules on the surface of scheelite particles is less complete than upon calcite and fluorite particles, and permits the replacement of the second layer of soap collector particles by a layer of the molecules of neutral oil which are strongly adsorbed by the first soap collector layer of particles and cause the selective flotation of scheelite.

It is noted that some siliceous material is floated along with the scheelite concentrate which floats in strongly agglomerated patches or clusters on the otherwise nearly clear froth. These clusters are air-bound and are held at the air-water interface. Since their apparent specific gravity is lower than that of the floated siliceous gangue, this latter undesirable contamination may be eliminated, and the scheelite concentrate upgraded by treating the froth carrying away the scheelite clusters by the method of agglomerate tabling.

In contradistinction to the conventional practice of tabling which is usually applied to recover materials too coarse to be levitated by froth flotation, the present invention resorts to tabling for the recovery of fine agglomerated scheelite which has been previously subjected to froth flotation, in a manner heretofore unknown in the art, as will be described later on in this specification. When the selective froth flotation of the ore in accordance with the process of the present in-

vention is followed by this tabling treatment of the agglomerated scheelite, the WO<sub>3</sub> content of the final concentrate is increased to a value as high as 40-50% by weight of WO<sub>3</sub> as compared with the values of 10% to 12% of WO<sub>3</sub> obtained by comparable froth flotation methods, e. g., using talol acids as collectors.

The operation of the process of this invention will be better understood by reference to the drawing, wherein: Figure 1 represents a flow diagram of the step-by-step processing of a typical tungsten-bearing ore in accordance with the invention; Figures 2 and 2A show diagrammatically a conventional shaking table; Figures 3 and 4 represent the stratification of the constituents of the pulp between the riffles and the distribution of materials as they come off the shaking table respectively in a conventional tabling treatment; Figures 5 and 6 illustrate the stratification of the pulp between the riffles and the distribution of materials leaving the table as in the present process.

In the flow diagram of Figure 1 the tungsten-bearing ore is fed to the process from mine 1 and undergoes a series of conventional crushing operations in a coarse crusher 2 and fine crusher 3, before being dumped into storage bin 4. The crushed ore is taken out from the storage bin and subjected to grinding (milling). Ordinarily, such an ore may contain copper in the form of chalcopyrite, molybdenum in the form of molybdenite and tungsten in the form of scheelite. The other constituents of the ore, the gangue, may comprise calcite, fluorite and a variety of siliceous minerals, chiefly quartz, epidote and garnet.

After wet grinding to a relatively coarse grind, for example, in a ball-mill 5, an aqueous pulp is formed which contains about 25% by weight of solids in the form of ore particles not larger than 35 mesh in size. This pulp proceeds to a conditioning tank 6 where it is conditioned with a mixture consisting of an appropriate conventional collecting reagent, such as an alkyl thiophosphate, for example, di-isobutyl dithiophosphate, or potassium amyl xanthate, in an amount of, say, 0.01 pound per ton of ore to float the chalcopyrite and, simultaneously, an adequate amount of pine oil or cresylic acid (e. g. 0.1 pound per ton of ore), or other suitable frothing agent for sulfide flotation, to act as a collector and frother for the molybdenite. In the diagram these conditioning agents are introduced into conditioner 6 from a mixing tank 10 via line 11.

Upon flotation in sulfide flotation cells 12 the combined sulfide concentrate or froth is sent through line 13 for additional processing, not shown in the diagram, to obtain separate chalcopyrite and molybdenite concentrates. This processing of sulfide-bearing froth may consist, for instance, in steaming to decompose the chalcopyrite collector and subsequently floating molybdenite away from chalcopyrite with the aid of additional frother, such as pine oil or cresylic acid, supplemented, if desired, by an addition of a small amount of neutral hydrocarbon oil of the white-oil type.

In order to recover scheelite by the process of selective froth flotation of the present invention, the tailings from the flotation of combined chalcopyrite-molybdenite concentrate are sent to another conditioning tank 14 to be treated with chemical reagents prior to beginning the flotation step. The conditioning treatment of the pulp formed by these tailings may be effected by forming a collector mixture in a mixing tank 15 and

introducing this mixture through line 16 into conditioning tank 14. The collector mixture in tank 15 comprises a naphthenic acid in the form of a soap, supplemented by a neutral hydrocarbon oil, the total amount of the oil in the mixture varying from about 20% to about 50% by weight based on the combined weight of the soap and oil. As mentioned hereinbefore, naphthenic acids effective as collectors in the flotation of scheelite have acid numbers ranging from about 160 to about 190 maximum (on oil-free basis) and their unsaponifiable hydrocarbon content may range from about 20% to about 50% by weight, provided the total content of neutral oil in the collector combination is less than about 50% by weight based on the combined weight of the oil-free acid and oil. Satisfactory selective flotation of scheelite is usually obtained by adjusting the pH of the pulp to a value of about 10.8 and upward prior to the introduction of naphthenic acid. Sodium carbonate and sodium hydroxide are ordinarily added as pH regulators. In addition, the scheelite collector mixture may comprise a slime regulator and depressant from siliceous materials, e. g., sodium silicate (specific gravity 40-41° Bé.), and a reagent, such as quebracho or a similar tannin-bearing material, to promote the depression of calcite, fluorite and siliceous gangue.

In a typical case, the following collector mixture may be used to condition the pulp prior to the flotation of scheelite:

|                                  | Lbs. per ton |
|----------------------------------|--------------|
| Sodium carbonate                 | 5.0          |
| Sodium hydroxide                 | 1.5          |
| Sodium silicate                  | 5.0          |
| Quebracho                        | 0.2          |
| Naphthenic acid (as sodium soap) | 1.5          |
| Neutral oil                      | 1.0          |

The conditioning treatment is effected by agitating the pulp with the reagents in tank 14 for at least 2 minutes in order to produce an intimate mixture, whereupon the pulp is fed into the rougher flotation cells 17.

The froth from these cells is directed into the cleaner flotation cells 20, while the rougher tailings, upon introduction of additional collector and, if desired, of neutral oil from tank 18 are sent to the middling flotation cells 21. Likewise, the tailings from the cleaner cells may be recycled as shown by line 22, if desired, to the rougher flotation cells 17. From the middling cells 21 the froth is recycled as shown by line 23 to be retreated in the rougher flotation cells 17, while the tailings are withdrawn to the reject pond.

The froth produced in the cleaner cells and carrying agglomerated clusters of scheelite may be contaminated with some siliceous gangue which failed to become depressed, in spite of the critical adjustment of pH to between 10.8 and 11.5 and the application of the novel collector combination of the present invention. In order to free the scheelite-bearing froth from these siliceous contaminants, it is subjected to agglomerate tabling.

This latter operation is effected by utilizing any type of conventional shaking table, as shown diagrammatically in Figures 2 and 2A. A typical table 24 may be 15 feet long and 5 feet wide at the narrow or concentrate end. Its deck is covered with linoleum or rubber and is given a slight inclination sidewise, as shown in Figure 2A. The riffling is  $\frac{1}{4}$ " wide, tapering from a depth of  $\frac{1}{2}$ " at the head and to a feather edge

along the diagonal line of termination and spaced  $1\frac{1}{2}$ " apart. The table has a reciprocating motion parallel to its long axis, variable from 230 to 280 strokes of about  $\frac{3}{4}$ " per minute. In the conventional tabling practice, the fine heavy mineral particles are deposited at the bottom between individual riffles, while coarse light mineral is deposited at the top and is sheared off during the tabling operation by the downflow of water, partly because of the thickening of the underlying bed of heavy mineral values between the riffles and partly because of the diminishing height of the riffles. The stratification obtained between the riffles and the distribution of the various materials as they leave the table in a conventional tabling operation are shown in Figures 3 and 4.

In the tabling step of the present invention, as shown in the flow diagram in Figure 1, the heavier tungsten values in the cleaner concentrate, agglomerated into air-bound flocks which are coarser and lighter than the gangue, are fed to shaking table 24. These flocks stratify at the top between the riffles, are entrained by the flow of wash water, and come off the tailing side of the table, as detailed in Figures 5 and 6. The resulting scheelite concentrate is subjected to drying in drier 25 and finally withdrawn to storage bin 26, while the siliceous tailings, if desired, may be returned to the rougher flotation cells, as shown by line 27.

The novel application of agglomerate tabling to the recovery of scheelite in accordance with the invention increases the  $WO_3$  content of the cleaner flotation concentrate by as much as 10% by weight, while the total recovery of scheelite from the original ore-feed by the present process is of the order of 90% by weight. Concentrates containing 40% to 50% and even more by weight of  $WO_3$  are readily produced by resorting to the particular collector combinations of the invention, maintaining the critical pH range of the pulp and further concentrating and recovering tungsten values by agglomerate tabling.

A number of small scale tests furnish the data which illustrate and emphasize the utility and advantages of the invention.

The ore used in these tests contained scheelite, calcite, fluorite, chalcopyrite and various siliceous minerals. Ore samples were crushed through No. 10 mesh in laboratory jaw crushers and rolls, and ground in a 12" ball mill at 50 R. P. M. Each ball mill charge of 500 g. of ore was ground for about 10 minutes with 300 cc. of water.

A typical screen analysis of such a ground ore is given below in Table I:

TABLE I

| Mesh    | Percent Retained |            |
|---------|------------------|------------|
|         | Direct           | Cumulative |
| 48      | 2.0              | 2.0        |
| 48-65   | 11.8             | 13.8       |
| 65-100  | 18.9             | 32.7       |
| 100-150 | 11.0             | 43.7       |
| 150-200 | 13.8             | 57.5       |
| 200     | 42.5             | -----      |

The mill feed analysis of this ore indicates the following content in mineral values:

$MoS_2$ -0.5%;  $Cu$ -0.3%;  $WO_3$ -0.35%

Flotation of chalcopyrite-molybdenite concentrate was effected in a 600 g. Fagergren laboratory cell having a rotor speed of 1800 R. P. M.,

dilution of the pulp being about 25% solids for both chalcopyrite-molybdenite and scheelite flotation. Chalcopyrite - molybdenite concentrate was floated away with the aid of a collector combination comprising an alkyl thiophosphate collector for chalcopyrite, such as di-isobutyl dithiophosphate (0.01 to 0.05 pound per ton), and pine oil acting as a collector and frother for molybdenite (0.1 to 0.15 pound per ton).

In the subsequent tests of molybdenite flotation, the effects of addition of various hydrocarbon oils on the grade of molybdenite concentrate were compared. Two neutral hydrocarbon oils were used: "A"—a heavy aromatic oil having an A. P. I. gravity of 13.9, and boiling between about 400° F. and about 700° F.; and oil "B"—obtained by polymerization of butenes and having a viscosity of about 222 S. S. U. at 210° F. The maximum of improvement in collection efficiency was noted in the case of a collector combination: di-isobutyl dithiophosphate (0.007 pound per ton), pine oil (0.12 pound per ton) and neutral oil "B" (1 pound per ton).

The results of these tests of molybdenite recovery are tabulated in Table II. The analyses of the concentrates and middlings were made by means of a polarograph, while those of the tailings by means of a spectrophotograph.

TABLE II  
*Effect of oils upon flotation of molybdenite*

|              | Concentrate    |                |                         | Tailing        |                |                         | Feed<br>Percent<br>Mo. |
|--------------|----------------|----------------|-------------------------|----------------|----------------|-------------------------|------------------------|
|              | Percent<br>Wt. | Percent<br>Mo. | Percent<br>Total<br>Mo. | Percent<br>Wt. | Percent<br>Mo. | Percent<br>Total<br>Mo. |                        |
| No Oil.....  | 1.31           | 10.4           | 65.5                    | 98.69          | 0.07           | 34.5                    | 0.21                   |
| Oil "A"..... | 1.44           | 10.6           | 68.8                    | 98.58          | 0.07           | 31.2                    | 0.22                   |
| Oil "B"..... | 1.13           | 11.6           | 52.4                    | 98.87          | 0.12           | 47.6                    | 0.25                   |

After the removal of the chalcopyrite-molybdenite concentrate the scheelite-bearing tailings were reconditioned for about two minutes with a mixture of the following reagents:

Lbs. per ton  
Sodium carbonate, a pH regulator ..... 5.0  
Sodium silicate (40° Bé), a slime regulator ..... 5.0  
Quebracho, a depressant for silicates and  
quartz ..... 0.5

Thereupon .75 pound per ton of oil-free naphthenic acid in the form of sodium soap was added to a similar batch of scheelite-bearing tailings, and the sample subjected to flotation in the rougher flotation cells.

The acid used in these tests has been originally

obtained by extraction of a lubricating oil fraction and contained about 43% by weight of unsaponifiable material; it was dissolved in dilute sodium hydroxide solution and repeatedly extracted with petroleum ether until substantially all saponifiable oils have been removed from it, whereupon it was acidified to yield an oil-free naphthenic acid having an acid number of approximately 177 and a specific gravity of 0.97. Upon withdrawing a rougher scheelite froth, an additional 0.75 pound per ton of oil-free naphthenic acid in the form of sodium soap was added to the rougher tailings and a middling froth removed from the corresponding flotation cells. The remaining material constituted the final rougher tailings. The rougher froth product was refloated in fresh water upon the addition of 0.25 pound per ton of naphthenic acid (as sodium naphthenate), and 1 pound per ton of sodium carbonate to yield a final cleaner concentrate. In this first test the pH of the pulp was equal throughout to 10.0. Two other tests, Nos. 2 and 3, were carried out at a higher pH of 11.2, which was achieved by the introduction of about 4 pounds per ton of sodium hydroxide prior to the recovery of rougher flotation froth and of additional 2 pounds per ton of sodium hydroxide prior to the recovery of final cleaner froth. In the last test, No. 3, the oil-free naphthenic acid (as sodium naphthenate) was applied together with about 0.75 pound per ton of neutral hydrocarbon oil, namely, a light petroleum fuel oil which boiled in the range from about 360° F. to about 684° F. and had a gravity value of 31.9° A. P. I., a flash point of 174° F., and a viscosity of 37.1 S. S. U. at 100° F. The cleaner froth product from all three tests was subjected to a form of agglomerate separation (tabling), by using a vanning plaque for the purpose, except in test No. 1 where the amount of cleaner froth was too small to permit separation.

The results of flotation tests Nos. 1, 2 and 3 are presented in Table III and indicate that a pH equal to 10.0, the application of oil-free naphthenic acid as a flotation agent results in a low recovery of  $WO_3$  equal to 50.8% by weight of the total  $WO_3$  in the ore, even though the cleaner concentrate grade is rather high (58.7% by weight of  $WO_3$ ). Increasing the pH to 11.2 depresses the scheelite and reduces both the concentrate grade and the total recovery, notwithstanding the application of agglomerate tabling. However, upon addition of neutral hydrocarbon oil in test No. 3, the concentrate grade was markedly improved and a very satisfactory recovery value of 61.9% was attained.

TABLE III

|                              | Test No. 1,<br>pH=10.0 Oil-free<br>Naphthenic Acid |                   |                            | Test No. 2,<br>pH=11.2 Oil-free<br>Naphthenic Acid |                   |                            | Test No. 3,<br>pH=11.2 Oil-free<br>Naphthenic Acid<br>and Neutral Oil |                   |                            |
|------------------------------|----------------------------------------------------|-------------------|----------------------------|----------------------------------------------------|-------------------|----------------------------|-----------------------------------------------------------------------|-------------------|----------------------------|
|                              | Percent<br>Weight                                  | Percent<br>$WO_3$ | Percent<br>Total<br>$WO_3$ | Percent<br>Weight                                  | Percent<br>$WO_3$ | Percent<br>Total<br>$WO_3$ | Percent<br>Weight                                                     | Percent<br>$WO_3$ | Percent<br>Total<br>$WO_3$ |
| Agglomerate Concentrate..... |                                                    |                   |                            | 0.61                                               | 21.5              | 32.2                       | 0.53                                                                  | 47.9              | 61.9                       |
| Agglomerate Tailing.....     | 0.21                                               | 58.7              | 50.8                       | 0.51                                               | 18.2              | 22.8                       | 0.20                                                                  | 37.4              | 18.4                       |
| Cleaner Concentrate.....     | 0.82                                               | 5.4               | 1.2                        | 2.12                                               | 1.4               | 1.4                        | 5.78                                                                  | 0.8               | 11.4                       |
| Cleaner Tailing.....         | 5.8                                                | .58               | 14.1                       | 11.2                                               | 0.35              | 9.6                        | 11.4                                                                  | 0.09              | 2.4                        |
| Middling.....                | 82.9                                               | .05               | 16.9                       | 81.4                                               | 0.14              | 28.0                       | 79.0                                                                  | 0.03              | 5.9                        |
| Rougher Tailing.....         | 10.3                                               |                   |                            | 4.2                                                |                   |                            | 3.1                                                                   |                   |                            |
| Heads.....                   |                                                    | 0.24              |                            |                                                    | .41               |                            |                                                                       | .41               |                            |

Another group of tests, Nos. 4, 5 and 6, were effected by following the same procedure as described for tests Nos. 1, 2 and 3. However, in these tests the naphthenic acid was a commercial grade naphthenic acid added in the form of sodium soap, having an acid number on oil-free basis equal to 173 and containing 30% by weight of unsaponifiable matter. The other reagents and test conditions were identical with those applied in tests 1, 2 and 3 except for the fact that 1.0 pound per ton of naphthenic acid was used to float the rougher and middling concentrates, instead of 0.75 pound per ton. The results presented in Table IV show that with the higher pH equal to 11.2, the application of commercial grade naphthenic acid containing about 30% by weight of unsaponifiable material as a flotation agent improves the recovery of scheelite as shown by the values determined for agglomerate concentrate. However, the addition of neutral oil to this acid in the amount of .75 pound per ton in test No. 6 showed very definitely that such an addition, bringing the total proportion of oil in the collector combination to a figure exceeding 50% by weight of the total weight of acid and oil, has an adverse effect on the recovery of scheelite.

TABLE IV

|                         | Test No. 4,<br>pH=10 Oil-Containing<br>Naphthenic Acid |                            |                                     | Test No. 5,<br>pH=11.2 Oil-Containing<br>Naphthenic Acid |                            |                                     | Test No. 6,<br>pH=11.2 Oil-Containing<br>Naphthenic Acid<br>+ Neutral Oil |                            |                                     |
|-------------------------|--------------------------------------------------------|----------------------------|-------------------------------------|----------------------------------------------------------|----------------------------|-------------------------------------|---------------------------------------------------------------------------|----------------------------|-------------------------------------|
|                         | Weight<br>Percent                                      | Percent<br>WO <sub>3</sub> | Percent<br>Total<br>WO <sub>3</sub> | Weight<br>Percent                                        | Percent<br>WO <sub>3</sub> | Percent<br>Total<br>WO <sub>3</sub> | Weight<br>Percent                                                         | Percent<br>WO <sub>3</sub> | Percent<br>Total<br>WO <sub>3</sub> |
|                         |                                                        |                            |                                     |                                                          |                            |                                     |                                                                           |                            |                                     |
| Agglomerate Concentrate | 0.06                                                   | 61.1                       | 14.8                                | 0.17                                                     | 54.9                       | 34.1                                | -----                                                                     | -----                      | -----                               |
| Agglomerate Tailing     | 0.04                                                   | 60.8                       | 9.6                                 | 0.08                                                     | 56.9                       | 16.9                                | -----                                                                     | -----                      | -----                               |
| Cleaner Concentrate     | -----                                                  | -----                      | -----                               | -----                                                    | -----                      | -----                               | -----                                                                     | -----                      | -----                               |
| Cleaner Tailing         | 0.77                                                   | 6.2                        | 19.2                                | 1.22                                                     | 2.9                        | 12.8                                | 0.09                                                                      | 12.4                       | 1.9                                 |
| Middling                | 2.12                                                   | 2.24                       | 19.2                                | 6.90                                                     | 0.66                       | 16.9                                | 0.27                                                                      | 4.9                        | 2.2                                 |
| Rougher Tailing         | 92.9                                                   | 0.10                       | 37.2                                | 89.0                                                     | 0.06                       | 19.3                                | 2.8                                                                       | 14.6                       | 60.1                                |
| Sulfide Concentrate     | 4.1                                                    | -----                      | -----                               | 2.6                                                      | -----                      | -----                               | 0.36                                                                      | 0.17                       | 26.8                                |
| Heads                   | -----                                                  | .25                        | -----                               | -----                                                    | .27                        | -----                               | 3.2                                                                       | -----                      | .59                                 |

In addition, tests were carried out with oleic acid (test No. 7) and semi-refined taloil acid (test No. 8), applied in the form of their sodium soaps, at a pH of 11.2 and with the addition of the same amount of the neutral hydrocarbon oil as used in preceding tests Nos. 4, 5 and 6. The test data presented in Table V show unambiguously that the improvement in the selectivity of scheelite flotation in the pH range from 10.8 to 11.5 are peculiar of the "naphthenic acid-neutral hydrocarbon oil" collector combination of the present invention and that fatty acids are unsuitable for the use in combination with such neutral oils.

TABLE V

|                         | Test No. 7<br>pH=11.2 Oleic Acid +<br>Neutral Oil |                            |                                     | Test No. 8<br>pH=11.2 Tallow Oil +<br>Neutral Oil |                            |                                     |
|-------------------------|---------------------------------------------------|----------------------------|-------------------------------------|---------------------------------------------------|----------------------------|-------------------------------------|
|                         | Percent<br>Weight                                 | Percent<br>WO <sub>3</sub> | Percent<br>Total<br>WO <sub>3</sub> | Percent<br>Weight                                 | Percent<br>WO <sub>3</sub> | Percent<br>Total<br>WO <sub>3</sub> |
|                         |                                                   |                            |                                     |                                                   |                            |                                     |
| Agglomerate Concentrate | 0.05                                              | 15.6                       | 1.4                                 | -----                                             | -----                      | -----                               |
| Agglomerate Tailing     | 0.05                                              | 28.4                       | 2.5                                 | -----                                             | -----                      | -----                               |
| Cleaner Concentrate     | -----                                             | -----                      | -----                               | 0.05                                              | 35.4                       | 3.1                                 |
| Cleaner Tailing         | 0.3                                               | 16.6                       | 9.0                                 | 0.92                                              | 34.3                       | 53.5                                |
| Middling                | 6.1                                               | 6.3                        | 69.1                                | 0.60                                              | 10.6                       | 10.8                                |
| Rougher Tailing         | 90.9                                              | 0.11                       | 18.0                                | 96.1                                              | 0.20                       | 32.6                                |
| Sulfide Concentrate     | 2.6                                               | -----                      | -----                               | 2.3                                               | -----                      | -----                               |
| Heads                   | -----                                             | 0.56                       | -----                               | 0.59                                              | -----                      | -----                               |

The data from the above tests clearly point out the superiority of the flotation results obtained

with the naphthenic acid-neutral hydrocarbon oil collective combinations, in which the proportion of neutral hydrocarbon oil, whether originally in the acid or subsequently added thereto, does not exceed 50% by weight based on the combined weight of the oil and acid, compared with the results obtained with naphthenic acid without neutral oil, or with a naphthenic acid-neutral oil combination containing neutral oil in excess of 50% by weight, or with a combination of a fatty acid or its soap with neutral oil.

The analysis of tungsten content as represented in the tabulated data was effected as follows: Ore samples were treated with an acid, preferably hydrochloric, in order to decompose scheelite and to precipitate most tungsten as tungstic acid. The remainder was filtered and washed and finally extracted with potassium hydroxide, the resulting potassium tungstate solution being thereafter acidified and treated with an excess of alpha benzoinoxime. The precipitated tungsten complex was filtered and ignited to WO<sub>3</sub>.

It has been observed that in certain instances, the efficiency of selective flotation according to the process of this invention may be adversely affected by the hardness of water used. Coarse and heavy flocks of tungsten mineral will then be

formed which will not respond satisfactorily to the tabling treatment and will cause a low recovery. A conventional softening treatment of the water to be used in the process will then remedy this condition. Generally speaking, the water to be used in the flotation process of the present invention will require softening whenever its hardness approaches about 88 p. p. m. of calcium ion.

The new process is not limited by the examples nor by the flow diagram described hereinabove, and includes within its scope all the modifications and variations thereof, except as limited by the appended claims. Thus, for example, the quanti-

ties of the various reagents may be varied to suit the requirements of each particular case;

likewise, the rougher concentrate may be cleaned and recleaned as many times as desired. Furthermore, other efficient collectors and frothers than pine oil and alkyl thiophosphates may be used for the recovery of copper and molybdenum values described hereinbefore.

In summarizing the various significant improvements over the prior art secured by this invention, the following important features thereof are emphasized:

(1) Production of high grade tungsten concentrates largely superior to those previously obtained in the art is now made possible;

(2) The grade of tungsten concentrate may be further improved by the application of agglomerate tabling to remove persisting siliceous contaminants;

(3) High amounts of tungsten minerals may be recovered from tungsten-bearing ores by selective flotation in the alkaline pH range of 10.8 to 11.5 with the aid of heavy naphthenic acids as flotation collectors improved by the addition of neutral hydrocarbon oil.

It is finally stressed that this invention is not limited to the flotation of scheelite away from calcite and fluorite, but that this process may also be successfully used to recover tungsten minerals from any type of tungsten-bearing ore, wherein other constituents have the same or an equivalent cation, such as calcium or magnesium and, therefore, cannot be floated away from each other by conventional flotation procedures. For instance, it is possible to separate scheelite from ores containing, e. g., scheelite and magnesite, or from ores containing scheelite, apatite and anhydrite.

As mentioned above, many modifications may be made in the process of the invention without departing from the spirit thereof, its scope being limited solely by the definitions in the appended claims.

I claim:

1. In a process of recovering scheelite from an ore pulp containing scheelite, calcite, fluorite and siliceous gangue and having a pH of between about 10.8 and about 11.5, the combination of steps of conditioning said pulp with sodium silicate as a slime regulator and a tannin-containing depressant for said calcite, fluorite, and siliceous gangue; effecting selective flotation of scheelite away from said calcite, fluorite, and siliceous gangue contained in said pulp in the presence of a collector combination comprising a soap of a naphthenic acid having an acid number on oil-free basis between about 160 and about 190 maximum, and further comprising from about 20% to less than about 50% by weight of a neutral petroleum hydrocarbon oil boiling between about 350° F. and about 700° F. and having a viscosity of less than about 55 S. S. U. at 100° F., based on the total weight of oil-free acid and oil.

2. In a process of recovering scheelite from an ore pulp containing scheelite, calcite, fluorite and siliceous gangue and having a pH of between about 10.8 and about 11.5, the combination of steps of conditioning said pulp with sodium silicate as a slime regulator and quebracho as a depressant for said calcite, fluorite, and siliceous

gangue; effecting selective flotation of scheelite away from said calcite, fluorite, and siliceous gangue contained in said pulp in the presence of a collector combination comprising a soap of a naphthenic acid having an acid number on oil-free basis between about 160 and about 190 maximum, and further comprising from about 20% to less than about 50% by weight of a neutral petroleum hydrocarbon oil boiling between about 350° F. and about 700° F. and having a viscosity of less than 55 S. S. U. at 100° F., based on the total weight of oil-free acid and oil.

3. In a process of recovering scheelite from an ore pulp containing scheelite, calcite, fluorite and siliceous gangue and having a pH of between about 10.8 and about 11.5, the combination of steps of conditioning said pulp with sodium silicate as a slime regulator and quebracho as a depressant for said calcite, fluorite and siliceous gangue; effecting said selective flotation of scheelite away from said calcite, fluorite and siliceous gangue contained in said pulp in the presence of a collector combination comprising a soap of a naphthenic acid having an acid number between about 160 and about 190 maximum on oil-free basis, and further comprising from about 20% to less than about 50% by weight of a neutral petroleum hydrocarbon oil boiling between about 350° F. and about 700° F. and having a viscosity of less than 55 S. S. U. at 100° F., based on the total weight of oil-free acid and oil; recovering the resultant supernatant float of light air-bound clusters of scheelite particles; and floating away said supernatant clusters of scheelite particles from the underlying heavier siliceous gangue of said float by agglomerate tabling.

WILLIAM A. BATES.

#### REFERENCES CITED

The following references are of record in the file of this patent:

#### UNITED STATES PATENTS

| Number    | Name            | Date          |
|-----------|-----------------|---------------|
| 1,319,129 | Wells           | Oct. 21, 1919 |
| 1,953,431 | Patek           | Apr. 3, 1934  |
| 2,069,365 | Handy           | Feb. 2, 1937  |
| 2,094,646 | Frantz          | Oct. 5, 1937  |
| 2,105,827 | Tartaron        | Jan. 18, 1938 |
| 2,120,485 | Clemmer et al.  | June 14, 1938 |
| 2,216,992 | Vogel-Jargensen | Oct. 8, 1940  |
| 2,303,962 | Tartaron et al. | Dec. 1, 1942  |
| 2,373,305 | Gieseke         | Apr. 10, 1945 |
| 2,395,639 | Monson          | Feb. 26, 1946 |
| 2,442,455 | Booth           | June 1, 1948  |
| 2,464,313 | Weinig          | Mar. 15, 1949 |

#### OTHER REFERENCES

Gaudin, Principles of Mineral Dressing (c), 1939, by McGraw-Hill Book Company, pages 387-388.

The Mineral Industry during 1939, vol. 48 (c), 1940, page 673.

Engineering and Mining Journal, April 1943, p. 66.

Taggart, Handbook of Mineral Dressing (c), 1945, section 12, page 13.